

1

2,786,787

**TEXTILE FABRIC RENDERED SOIL RESISTANT  
WITH ALUMINUM PHOSPHATE AND METHOD  
OF PRODUCING SAME**

Patrick A. Florio, Elmhurst, N. Y., assignor to Mohasco Industries, Inc., a corporation of New York

No Drawing. Application April 13, 1954,  
Serial No. 422,987

12 Claims. (Cl. 117—169)

This invention relates to the treatment of surfaces to reduce the adherence or attraction of particles thereto and more particularly to the treatment of fabrics, paper and paper-like materials, paint films and other materials to reduce their color change due to pick-up and retention of particles on their exposed surfaces.

A more specific object is to reduce color change or greying of fabrics (flat or pile), covering or wrapping material, such as paper, and films, such as paint or varnish, due to the pick-up and retention of particles during use.

Another object is to reduce the particle adherence of surfaces without introducing an undesirable discoloration or whitening or otherwise harmfully altering the appearance or feel of the treated material.

Another object is to reduce the adherence of soil particles to surfaces.

Other objects and advantages will be apparent as the nature of the invention is more fully disclosed.

The treatment in accordance with this invention comprises depositing on the surface to be protected a composition containing aluminum phosphate and having characteristics which make it effective for the purpose as illustrated by the specific examples.

The composition may be applied to the surface from a dispersion under conditions to leave a coating of the desired weight and composition after the vehicle has been removed.

The surface can be treated in various ways depending upon its type and the results desired. In the case of pile fabrics, such as rugs or carpets, a water dispersion of the composition may be sprayed over the pile surface in an amount to produce the desired particle pick-up, or the dispersion may be applied by means of a carpet cleaning brush and then dried, or the fabric may be inverted and the pile only dipped into the dispersion. When used as a part of a standard rug-making process the dispersion may be sprayed onto the pile (face up) or the pile dipped (face down) after sizing and the treated rug then passed through a standard drier for removing the vehicle. If the treatment is applied to a carpet on the floor it may be dried at room temperature by allowing it to stand for a sufficient period of time.

After drying the coating has the property of adhering strongly to the surface. If eventually removed as a result of repeated cleaning or use it can be easily renewed.

The treatment is effective on various textiles such as wool, cotton, jute, viscose rayon, acetate rayon, nylon, acrylics, polyesters, and other synthetic fibers and/or blends thereof.

Rugs having pile composed of wool yarn or a synthetic yarn or of blends thereof, such as wool and rayon or wool and nylon may be treated by spraying the dispersion, preferably in the form of a fine mist and then drying.

Cotton pile rugs may be immersed in the dispersion until the desired pick-up has taken place on the fibers. The fabric is then passed between squeeze rollers and dried to leave the desired coating on the pile.

2

The dispersion may be applied to wall paper or to a surface by spraying or painting technique and allowed to dry at room temperature to form a coating having the characteristics above described.

5 The treatment is suited in general for any surface which is subject to particle adherence.

In accordance with this invention a dispersion of aluminum phosphate ( $\text{AlPO}_4$ ), a water insoluble phosphate of extremely small particle size, in salt free water 10 as a vehicle is applied to the surface by dipping, spraying or by other known techniques to leave after drying a coating of aluminum phosphate on the surface. The aluminum phosphate may be mixed with other materials as set forth in the examples.

15 Treatment according to the following examples has been found to improve the soil resistance of the treated surfaces without undesirable whitening or other discoloration and without increasing the harshness or otherwise changing the feel of the material.

20

*Example 1*

A dispersion made by mixing 1 part of aluminum phosphate ( $\text{AlPO}_4$ ) of extremely small average particle size (70 millimicrons and below) in 99 parts of salt free 25 water, was stirred vigorously for a period of 10 minutes. A pile fabric having 22 ounces per square yard of pile fiber was treated by immersion face down in this dispersion at room temperature to produce a solids pick-up of 1% on a dry basis on the pile weight. This corresponds to a pick-up of 0.011 ounce per square yard of exposed fiber surface area.

*Example 2*

A dispersion made by mixing 1 part of aluminum phosphate ( $\text{AlPO}_4$ ) of extremely small average particle size (70 millimicrons and below) and 0.25 part of trisodium phosphate ( $\text{Na}_3\text{PO}_4 \cdot 12\text{H}_2\text{O}$ ) and 98.75 parts of salt free water was sprayed at room temperature as a fine mist onto the pile surface of an Axminster pile carpet having a 35 backing composed of cotton chain and filler yarns, jute stuffer yarns and one-half inch pile having a weight of 23.2 ounces per square yard composed of a blend of 50% wool and 50% rayon. The pH of the pile may be 4 to 6.5. The spray may be controlled so that the weight of the dispersion taken up by the pile is about 100% of the 40 pile weight and is concentrated on the pile with the backing remaining substantially dry. The carpet is then passed through a drier at a temperature of about 175° F. to remove the water and leave a coating of aluminum phosphate on the pile of about 1% by weight of the pile, 45 corresponding to about .011 ounce per square yard of exposed fiber surface area. The coating is most concentrated at the free ends of the pile although some of the coating may extend down to the portion of the pile anchored in the backing.

55

*Example 3*

A dispersion made by mixing 1 part of aluminum phosphate ( $\text{AlPO}_4$ ) of extremely small average particle size (70 millimicrons and below), 0.25 part of trisodium phosphate,  $\text{Na}_3\text{PO}_4 \cdot 12\text{H}_2\text{O}$ , 0.25 part of Carbowax (a polyethylene glycol high molecular weight wax made by Carbide and Carbon Chemicals Corporation), and 98.75 parts of salt free water, was applied to the exposed fiber surface of a pile fabric containing a blend of carpet 60 wool and viscose rayon by spraying at room temperature. After drying, a pick-up of 1% aluminum phosphate on the pile or .011 ounce per square yard of exposed fiber surface was obtained.

*Example 4*

65 A dispersion was made by mixing 0.5 part of aluminum phosphate, 0.25 part of trisodium phosphate, and 0.25

part of Carbowax into 99.00 parts of salt free water. The mixture was stirred vigorously for 10 minutes. This dispersion was used to treat carpet as above.

*Example 5*

Other materials may be added to the dispersion in order to improve the soil repellency qualities. For example, a dispersion was made by mixing 0.5 part of aluminum phosphate, 0.25 part of Ludox (a silicon oxide sold by Du Pont), 0.25 part of trisodium phosphate, 0.25 part of Carbowax, and 98.75 parts of salt free water. The mixture was stirred vigorously for a period of 10 minutes. The dispersion was used to treat carpet as in Examples 1 to 3.

Other metal oxides may be used in place of Ludox, such as Alon, an aluminum oxide sold by Godfrey Cabot, Inc., aluminum aerogel, titanium oxide, etc. Representative water dispersions of these materials are set forth in the following table:

ALUMINUM PHOSPHATE AND METAL OXIDES

[Oxides in water dispersion for use in the treatment of pile carpet as set forth in Example 1.]

| Parts AlPO <sub>4</sub> | Parts Metal Oxides                          | Parts TSP | Parts Carbowax |
|-------------------------|---------------------------------------------|-----------|----------------|
| 0.25                    | 0.25 Alon (Al <sub>2</sub> O <sub>3</sub> ) | 0.25      | 0.25           |
| 0.50                    | 0.25 TiO <sub>2</sub> (Titanox)             | 0.25      | 0.25           |
| 0.50                    | 0.25 hydrous alumina                        | 0.25      | 0.25           |
| 0.25                    | 0.25 hydrous silica                         | 0.25      | 0.25           |

*Example 6*

Organic film-forming materials can likewise be added to improve the soil resistance properties. For example, a dispersion was made by mixing 0.5 part of aluminum phosphate, 0.25 part of methocel (carboxy methyl cellulose sold by Dow Chemical), 0.25 part of trisodium phosphate, 0.25 part of Carbowax, with 98.75 parts of salt free water. This mixture was stirred and used to treat carpet as in Examples 1 to 3.

*Example 7*

A combination of oxides may be used to aid the aluminum phosphate in giving soil resistance. For example, a dispersion was made by mixing 0.5 part of aluminum phosphate, 0.25 part of Alon, 0.25 part of Ludox, 0.25 part of trisodium phosphate, 0.25 part of Carbowax, and 98.5 parts of salt free water. This dispersion was used to treat carpet as in Examples 1 to 3.

*Example 8*

Other water insoluble inorganic materials having particle sizes of a colloidal nature such as silicates and clays may also be used as an addition to the aluminum phosphate to improve its soil resistance properties. For example, a dispersion may be made by mixing 0.5 part of aluminum phosphate, 0.25 part of Veegum (an aluminum magnesium silicate made by the Vanderbilt Co.), 0.125 part of trisodium phosphate, 0.125 part of Carbowax, and 99 parts of salt free water. This mixture was stirred vigorously and used to treat carpet as in Example 1.

*Example 9*

A dispersion prepared as set forth in the above examples and containing .5% solids may be applied by a brush to a standard wall paper while on the wall and to a painted surface in a quantity to produce a solids coating of .01 ounce per square yard.

*Example 10*

A flat non-pile fabric (flag bunting, weight 4.75 ounces per square yard) may be passed through a dispersion prepared as set forth in the above examples and between squeeze rollers to leave a solids pick-up of from 1% to 1.5% by weight when dry, corresponding to about .0091

ounce to .0137 ounce per square yard of exposed fiber surface area.

*Example 11*

A dispersion in an organic vehicle may be made by adding one part aluminum phosphate to 100 parts of isopropanol or of ethyl alcohol containing from 1% to 10% water. This dispersion can be used as in any of the previous examples.

Other volatile organic vehicles that can be used are:

Methanol  
Acetone  
Ethylene glycol  
Carbon tetrachloride

Additions may be made to the AlPO<sub>4</sub> dispersion to satisfy the need for other properties such as (1) lowering whitening effect by the addition of metal oxides; (2) improvement of hand by the addition of known softening agents; and (3) improvement of color change by the addition of dyes or other coloring matter.

In any of the above examples other known wetting and dispersing agents may be used in place of the trisodium phosphate, or, if desired, the wetting or dispersing agent may be omitted.

Also other waxes may be used in place of the Carbowax for improving the hand and decreasing the harshness of the treated surface or the wax may be omitted if not required for a particular purpose.

The spraying or dipping may be controlled so that the desired weight of coating is formed.

A coating of .5% to 1.5% dry solids based on the weight of the pile has been found most effective for many types of pile materials although the coating may be varied from .25% to 5% for some purposes. An excess of the composition may be used but usually does not further decrease the adherence of soil particles and may increase the whitening effect. In addition it may result in excess dusting and may become noticeable in the feel of the material.

The surface area of fiber coated may be calculated by the following equation:

$$A_s = W \times \frac{1}{D} \times \frac{4}{d_f} \times F$$

Where W equals the total weight of fiber per square yard; A<sub>s</sub> equals the effective exposed fiber surface area (in square yards) per square yard of fabric; D equals average density of the fiber in pounds per cubic yard calculated by (specific gravity)  $\times 1685$ ; d<sub>f</sub> equals average diameter of the fiber in yards calculated by (fiber diameter in microns)  $\times 1.095 \times 10^{-6}$ ; and F equals a factor showing the average degree of penetration of the treating dispersion expressed as a fraction of the total fiber area which is coated.

F values of from one-third to one-twelfth may be used, depending upon yarn construction, coating technique, fiber diameter, and fabric construction.

While in general the weight of coating varies from 0.25 percent to 5.0 percent of the fabric weight, the amount of material applied per square yard of exposed fiber surface may vary from .003 to .054 ounce per square yard of exposed fiber surface area computed as above. A range of .0063 to .024 ounce per square yard of exposed surface usually produces satisfactory results.

For flat surfaces such as paint film or paper and the like these same limits in ounces of coating per square yard apply.

If pile surfaces are treated by spraying or dipping the major part of the coating is deposited on the exposed pile tufts toward the free ends thereof although some of the composition may migrate to the bound portions of the pile and to the backing.

Standard detergents, wetting and dispersing agents may be used with the above dispersions if desired. These are

particularly useful to effect a combination of cleaning and treating.

Obviously the above treatment can be applied to fibers prior to spinning, to yarn prior to weaving or to fabrics after weaving.

What is claimed is:

1. A textile fabric having a surface coating of discrete, pre-formed aluminum phosphate, the average particle size of said aluminum phosphate being not greater than about 70 millimicrons, the coating being present on the material in an amount of from about 0.25% to about 5% of the weight of the fabric, said coating having the property of reducing the tendency of the surface to pick up and retain soil particles.

2. A textile fabric as set forth in claim 1 having a backing and pile elements anchored therein, the pile elements forming the exposed surface and having the coating of the particles of aluminum phosphate.

3. A textile fabric as set forth in claim 1 in which the surface coating includes a softening agent.

4. A textile fabric as set forth in claim 1 in which the coating also includes a finely-divided metal oxide.

5. A textile fabric as set forth in claim 1 in which the metal oxide is aluminum oxide.

6. A textile fabric as set forth in claim 1 in which the metal oxide is silicon oxide.

7. The method of reducing the particle adherence characteristics of a textile fabric without producing an undesirable color change therein, which comprises applying to a surface of said fabric a dilute liquid dispersion containing pre-formed particles of aluminum phosphate having an average particle size not greater than about 70

millimicrons, and removing the dispersion vehicle from the fabric, the amount of dispersion applied to the surface being such as to leave thereon an amount of the aluminum phosphate equal to about 0.25% to about 5% of the weight of the fabric.

5 8. The method of claim 7 in which the dispersion of the aluminum phosphate includes a wetting and dispersion agent.

9. The method of claim 7 in which the dispersion of aluminum phosphate includes a softening agent.

10 10. The method of claim 7 in which the dispersion of aluminum phosphate also includes a finely-divided metal oxide.

11. The method of claim 10 in which the metal oxide is aluminum oxide.

15 12. The method of claim 10 in which the metal oxide is silicon oxide.

#### References Cited in the file of this patent

##### UNITED STATES PATENTS

|              |                      |               |
|--------------|----------------------|---------------|
| 20 1,434,549 | Lewis et al. -----   | Nov. 7, 1922  |
| 1,983,349    | Dreyfus -----        | Dec. 4, 1934  |
| 2,033,977    | Dreyfus -----        | Mar. 17, 1936 |
| 2,230,656    | Scholler -----       | Feb. 4, 1941  |
| 25 2,570,750 | Bauer -----          | Oct. 9, 1951  |
| 2,587,505    | Moody -----          | Feb. 26, 1952 |
| 2,622,307    | Cogovan et al. ----- | Dec. 23, 1952 |

##### OTHER REFERENCES

30 Synthetic Organic Chemicals, 12th edition, July 1, 1946, pages 22 and 23, Carbide and Carbon Chemicals Corp.